

## UNITED STATES PATENT OFFICE

2,186,447

METHOD OF MAKING MOLYBDENUM AND  
ALLOYS OF MOLYBDENUMJoseph H. Brennan, Niagara Falls, N. Y., assignor  
to Electro Metallurgical Company, a corpora-  
tion of West VirginiaNo Drawing. Application January 28, 1939,  
Serial No. 253,449

4 Claims. (Cl. 75—176)

The principal ores of molybdenum, including the sulfide ore, molybdenite, very often contain substantial amounts of copper minerals, for instance copper sulfide, which can not readily be separated from the ore by mechanical methods. Inasmuch as there is a demand for metallic molybdenum and molybdenum alloys containing one or more metals of the iron group (iron, cobalt, nickel) with little or no copper, a practical method is needed for producing these alloys from copper-contaminated molybdenite, roasted molybdenite, or other molybdenum sources. It is an object of this invention to provide such a process.

15 In accordance with the invention, molybdenite, roasted molybdenite, or other ore source of molybdenum, contaminated with copper mineral, is reacted with a reducing agent in the presence of a basic flux essentially containing sodium sulfide. Metal of the iron group may be added before, during, or after the main reaction, either as a mixture of metal compound and reducing agent or as reduced metal, or in both forms. Practically all of the copper originally associated with the 20 ore dissolves in the flux as copper sulfide and is retained therein.

25 Carbonaceous material, for instance bituminous coal, is an inexpensive and wholly satisfactory reducing agent, although other reducing agents may be used. A moderate excess of reducing agent is desirable, but a large excess should be avoided.

30 Soda ash is a satisfactory form of basis flux for use in this process. The sodium carbonate is believed to enter into a chemical reaction of the type:



35 thereby supplying sodium sulfide to the slag. A substantial excess of sodium carbonate may be used. Lime, limestone, magnesia, or dolomite may be added to supplement the action of sodium carbonate by reactions of the type:



40 and to aid in fluxing gangue materials, silicate for instance. Other basic, or neutral, fluxing agents may be added if desired. Preferably, a rather large excess of basic fluxes is added to keep the slag basic. It is preferred, furthermore, that sodium be the predominating base-forming element of the slag.

45 As indicated above, the sodium sulfide may be formed by reaction of soda ash with carbon and the sulfides in the ore. Alternately or addition-

ally, sodium sulfide may be added to the slag; or sodium sulfate and a reducing agent; or calcium sulfate, a reducing agent, and a sodium compound such as soda ash. The latter methods are particularly useful in the treatment of oxidized ores of molybdenum.

5 The molybdenite material to be treated will ordinarily contain between 25% and 60% molybdenum and 1% to 15% copper.

10 The following specific examples of processes embodying the principles of the invention serve to illustrate such principles, but it will be understood that the scope of the invention is not limited to or by these examples.

## Example I

15

100 parts of a molybdenite concentrate containing 34.2% Mo, 3.5% Fe, 1.5% Cu, 25% S, remainder chiefly gangue, was mixed with 100 parts of soda ash, 50 parts of lime, 29 parts of iron (nail scrap), and 27 parts of bituminous coal. The mixture was melted in an open-arc electric furnace, the reactions completed, the slag removed, and the alloy cast. The cast alloy contained 53.2% Mo, 1.6% C, 0.13% Cu, 0.24% S, remainder iron. Thus, the ratio of Mo to Cu of 20 about 22 in the ore was raised to about 400 in the alloy. The slag contained 2.98% Mo and 0.45% Cu.

## Example II

30

100 parts of molybdenite concentrates containing 28.2% Mo, 10.9% Cu, 10.9% Fe, 31.0% S, remainder chiefly gangue (ratio of Mo to Cu about 2.6) was mixed with 72 parts of soda ash, 65 parts of lime, 10 parts of iron (nail scrap), and 25 parts of bituminous coal. The mixture was melted and treated as in Example I. The resulting alloy contained 69.6% Mo, 27.4% Fe, 1.4% Cu, 0.19% C, and less than 0.08% S (a ratio of Mo to Cu of about 49). The slag contained 40 about 5% each of molybdenum and copper.

## Example III

100 parts of the same concentrate as that used in Example II was mixed with 75 parts of soda ash, 65 parts of lime, 13 parts of iron (nail scrap), and 35 parts of bituminous coal. From reduction as in the previous examples, an alloy was obtained containing 61% Mo, 34.8% Fe, 2.8% Cu, 0.29% S, and 0.18% C (ratio of Mo to Cu about 21.7).

45 Modifications may be made in the above-described procedure without departing from the invention. For instance, sodium compounds 50

55

other than sodium carbonate may be used, and heating means other than an open-arc electric furnace may be utilized. However, the preferred procedure is that specifically described herein.

5 5 I claim:

- 10 10 1. Method of treating crude material containing reducible compounds of molybdenum and copper to produce a molybdenum alloy in which the ratio of molybdenum to copper is higher than in said crude material, which includes the step of reducing said compounds in the presence of a basic flux essentially containing sodium sulfide.
- 15 15 2. Method of making, from molybdenite material containing a substantial proportion of copper as copper sulfide, a molybdenum alloy in which the ratio of molybdenum to copper is higher than in said molybdenite material, which comprises reducing said molybdenite material in the presence of a basic slag essentially containing sodium sulfide.

3. Method of making, from molybdenite material containing a substantial proportion of copper sulfide, molybdenum alloys in which the ratio of molybdenum to copper is higher than in said molybdenite material, which comprises heating at a reaction temperature a mixture including said molybdenite material, coal, soda ash, and lime, and coalescing the resulting metallic molybdenum with molten metal of the iron group.

4. Method which comprises melting in an electric furnace a mixture consisting of the following ingredients in approximately the proportions indicated: molybdenite containing 25% to 60% molybdenum and about 1% to 15% copper, 100 parts; bituminous coal, 25 to 35 parts; soda ash, 70 to 100 parts; lime, 50 to 65 parts; iron, 10 to 30 parts; and separating the resulting low-copper alloy and high-copper slag.

JOSEPH H. BRENNAN. 20